

## UNITED STATES PATENT OFFICE

2,380,280

## CHEMICAL SENSITIZING OF EMULSIONS

Walter J. Weyerts, Rochester, N. Y., assignor to  
Eastman Kodak Company, Rochester, N. Y., a  
corporation of New Jersey

No Drawing. Application March 6, 1943,  
Serial No. 478,303

12 Claims. (Cl. 95—7)

This invention relates to photographic emulsions and particularly to a method for increasing the speed of such emulsions.

The chemical sensitizing of photographic emulsions relates to increasing the speed of an emulsion in the region to which it is sensitive without appreciably increasing the optical range of sensitization. Agents used for this purpose have consisted for the most part in compounds of elements of the sulfur group and bio-chemical extracts. The present invention relates to a new class of compounds for the purpose of increasing the speed of photographic emulsions.

I have found that photographic emulsions of the silver halide type may be treated with water-soluble salts of unsaturated lower aliphatic acids for the purpose of increasing the speed or sensitivity.

Compounds suitable for this purpose are the water-soluble salts of unsaturated lower aliphatic acids. These include monobasic acids such as acrylic acid, methacrylic acid, benzoyl acrylic acid, furoyl acrylic acid and crotonic acid, and dibasic acids such as itaconic acid, citraconic acid, and maleic acid. Water-soluble salts of these acids which may be employed are the sodium, potassium and ammonium salts.

The degree of increase in sensitivity obtained has been found to vary with the type of emulsion employed and with the nature and quantity of salt added. The addition agents of my invention may be employed with non-optically sensitized gelatino-silver halide emulsions or with emulsions sensitized with optical sensitizing dyes in the customary manner. In some instances the increase in speed of the emulsion was accompanied by a change in contrast as well, while in other cases little or no change in contrast was noted.

Suitable compounds for increasing the speed of

silver halide emulsions according to my invention are the following:



Sodium acrylate



Sodium methacrylate



Sodium crotonate



Sodium benzoylacrylate



$\alpha$ -furyl sodium acrylate



Sodium itaconate



Sodium citraconate



Sodium maleate

My invention will be illustrated by reference to the following specific examples, in which the speed is expressed as ten times the reciprocal of the inertia.

*Example 1*

A moderately coarse grained bromoiodide emulsion which had a speed of 575, a gamma of 1.29 and a fog level of 0.06 was compared with a simi-

lar emulsion to which had been added 10 grams per liter of emulsion of sodium acrylate. The emulsion to which the sodium acrylate had been added showed a sensitivity increase of about 60% without an appreciable increase in the gamma or fog level. The emulsions compared as follows:

|                                           | 10/i<br>speed | Gamma | Fog |
|-------------------------------------------|---------------|-------|-----|
| Check.....                                | 575           | 1.29  | .06 |
| Emulsion with 10 g. sodium acrylate/liter | 920           | 1.55  | .07 |

Both emulsions were developed for 4 minutes in the following developing solution:

|                                       |         |
|---------------------------------------|---------|
| Monomethyl-p-aminophenol sulfate..... | 2.2     |
| Hydroquinone.....                     | do 8.8  |
| Sodium sulfite (desiccated).....      | do 96   |
| Sodium carbonate (desiccated).....    | do 48   |
| Potassium bromide.....                | do 5    |
| Water to.....                         | liter 1 |

#### Example 2

A high speed optically sensitized emulsion of medium fine grain having a speed of 1320, a gamma of 0.74 and a fog level of 0.05 was compared with similar emulsions in which sodium acrylate and sodium methacrylate had been added in the amount of 10 grams per liter of emulsions. A speed increase was noted as shown in the following table:

|                                                    | 10/i  | Gamma | Fog |
|----------------------------------------------------|-------|-------|-----|
| Check.....                                         | 1,320 | 0.75  | .05 |
| Emulsion with 10 g. sodium acrylate/liter.....     | 1,910 | 0.73  | .06 |
| Emulsion with 10 g. sodium methacrylate/liter..... | 2,820 | 0.65  | .16 |

The emulsions were developed for 12 minutes in the following developing solution:

|                                       |         |
|---------------------------------------|---------|
| Monomethyl-p-aminophenol sulfate..... | 2       |
| Hydroquinone.....                     | do 5    |
| Sodium sulfite (desiccated).....      | do 100  |
| Borax.....                            | do 2    |
| Water to.....                         | liter 1 |

#### Example 3

An optically sensitized gelatino-silver bromide emulsion having a speed of 1150, a gamma of 0.74 and a fog level of 0.05 was compared with a similar emulsion to which 5 grams of sodium methacrylate had been added per liter of emulsion. The results are shown in the following table:

|                                                   | 10/i<br>speed | Gamma | Fog |
|---------------------------------------------------|---------------|-------|-----|
| Check.....                                        | 1,150         | .74   | .05 |
| Emulsion with 5 g. sodium methacrylate/liter..... | 1,910         | 0.73  | .07 |

The emulsions were developed in the developing solution of Example 2.

While I prefer to use my addition agents in the amount of approximately 10 to 20 grams per liter of wet emulsion, the amounts used may be as low as 5 grams per liter or as great as 25 grams per liter. The degree of increase in sensitivity obtained depends upon the quantity of the addition agent used. With these agents the speed increase

varies from 25% to 100% or more depending upon the type of emulsion and the nature and quantity of the salt added.

While my addition agents will generally be used with gelatino-silver halide emulsions, such as emulsions of the bromide or bromo-iodide type, they may also be used with silver halide emulsions in which the carrier is albumen, collodion or other cellulose ester or synthetic resin, provided that there is considerable water in the emulsion to act as a solvent for the addition agent.

It will be understood that the above examples are illustrative only and that my invention is to be taken as limited only by the scope of the appended claims.

#### I claim:

1. The method of increasing the speed of a silver halide photographic emulsion, which comprises adding thereto from 5 to 25 grams per liter of a water-soluble salt of an unsaturated, lower aliphatic acid.

2. The method of increasing the speed of a silver halide photographic emulsion, which comprises adding thereto from 5 to 25 grams per liter of the sodium salt of an unsaturated, lower aliphatic acid.

3. The method of increasing the speed of a silver halide photographic emulsion, which comprises adding thereto from 5 to 25 grams per liter of a water-soluble salt of an unsaturated, lower aliphatic acid.

4. The method of increasing the speed of a silver halide photographic emulsion, which comprises adding thereto from 5 to 25 grams per liter of the sodium salt of an acrylic acid.

5. The method of increasing the speed of a gelatino-silver halide emulsion, which comprises adding thereto the sodium salt of acrylic acid in an amount sufficient to effect an appreciable sensitivity increase.

6. The method of increasing the speed of a gelatino-silver halide emulsion, which comprises adding thereto the sodium salt of methacrylic acid in an amount sufficient to effect an appreciable sensitivity increase.

7. A gelatino-silver halide emulsion containing as a speed-increasing agent from 5 to 25 grams per liter of a water-soluble salt of an unsaturated, lower aliphatic acid.

8. A gelatino-silver halide emulsion containing as a speed-increasing agent from 5 to 25 grams per liter of the sodium salt of an unsaturated, lower monobasic acid.

9. A gelatino-silver halide emulsion containing as a speed-increasing agent from 5 to 25 grams per liter of the sodium salt of an acrylic acid.

10. A gelatino-silver halide emulsion containing as a speed-increasing agent from 5 to 25 grams per liter of the sodium salt of acrylic acid.

11. A gelatino-silver halide emulsion containing as a speed-increasing agent approximately 10 grams per liter of wet emulsion of sodium acrylate.

12. A gelatino-silver halide emulsion containing as a speed-increasing agent approximately 10 grams per liter of wet emulsion of sodium methacrylate.

WALTER J. WEYERTS.